

## UNITED STATES PATENT OFFICE

2,322,084

SIMULTANEOUS BLEACHING AND FIXING  
BATH

Richard V. Young and Merrill W. Seymour,  
Rochester, N. Y., assignors to Eastman Kodak  
Company, Rochester, N. Y., a corporation of  
New Jersey

No Drawing. Application November 6, 1940, Serial  
No. 364,548. In Great Britain January 11,  
1940

8 Claims.

(Cl. 95—6)

This invention relates to improvements in color photography and more particularly in processes wherein dyes present in a silver halide emulsion are bleached in the vicinity of a silver image.

It is known that the bleaching of dyes selectively in the neighborhood of a silver image can be accomplished by reagents such as acid thiourea. It is possible to control the contrast of the dye images by the addition of azo dyes or other mild oxidizing agents to the bleaching solutions which cause less image-forming dye to be reduced by a given amount of silver for the available reducing agent because they compete with the azo dyes present in the emulsion, as described in our application Serial No. 355,098 filed August 31, 1940. This lowers the contrast of the dye images.

In the processes of the bleaching-out type, it has hitherto been customary to fix out the undeveloped silver salts before treatment with the bleach baths. In such bleaching-out processes, moreover, there is generally some excess of silver left behind after the bleaching of the dye has been carried to the desired point. This residual silver has to be removed after oxidation with some reagent which does not destroy the dye images, such as a solution of cupric chloride. The treatment of photographic elements by the bleaching-out process therefore generally involves five operations, apart from the necessary washing steps, namely: (1) development; (2) fixing out the undeveloped silver halide; (3) dye-bleaching; (4) oxidation of the residual silver to a silver salt; (5) fixing out the silver salt.

It has now been found possible to employ a bleach bath which will simultaneously accomplish operations (2), (3), (4) and (5), rendering unnecessary any separate operation for fixing out residual silver halide and for removing unused silver. By reduction in the number of chemical operations it is also possible to reduce the number of washes and this accomplishes a great saving in time.

According to the present invention, therefore, in a photographic dye bleach-out process there is used a bleaching bath which contains a fixing agent for silver halide and a mild oxidizing agent which serves to oxidize any silver remaining after the bleaching of the dye.

In such a bath the undeveloped silver halide is fixed out, the dye is bleached, the silver is oxidized and the oxidation product of the silver is fixed out in one operation, provided that a suitable quantity of the mild oxidizing agent is employed. The presence of the mild oxidizing agent also makes it possible to effect control of the gamma of the dye image since the relative con-

centrations of the oxidizing agent and of the other constituents of the bleach bath may be altered as required to bleach the desired amount of dye in the time necessary to oxidize all of the silver

5 to a soluble silver complex.

The invention includes a bleach bath for use in a dye bleach-out process containing a fixing agent, a strong acid and a mild oxidizing agent capable of oxidizing metallic silver to a silver

10 salt.

Any mineral acid may be used as a strong acid, such as hydrochloric acid, hydrobromic acid, hydroiodic acid, nitric acid, and phosphoric acid. Among oxidizing agents which can be used may be mentioned ferric chloride, ammonium vanadate, vanadyl chloride, potassium ferricyanide, potassium nitrate and organic compounds such as soluble nitro and nitroso compounds and azo dyes which can rapidly diffuse into and out of an emulsion.

20 Examples will now be given of suitable bleaching baths for carrying out the present inventions:

## Example 1

|    |                          |                   |       |
|----|--------------------------|-------------------|-------|
| 25 | Potassium thiocyanate    | grams             | 12    |
|    | Oxyamino phenazine       | do                | 0.004 |
|    | Hydrochloric acid, conc. | cubic centimeters | 5     |
|    | Dimethyl quinoxaline     | grams             | 0.02  |
| 30 | Ferric alum              | do                | 0.1   |
|    | Water, to                | cubic centimeters | 100   |

In this solution, the thiocyanate ion is responsible for the fixing and for the formation of a soluble complex of silver when the silver becomes oxidized. The complex formed from the thiocyanate and ferric ions acts as the mild oxidizing agent to oxidize the silver not oxidized by the bleaching of the image-forming dye. The oxyamino phenazine and the dimethyl quinoxaline act as a bleaching catalyst.

## Example 2

|    |                                        |                   |       |
|----|----------------------------------------|-------------------|-------|
| 45 | Potassium thiocyanate                  | grams             | 14.0  |
|    | H <sub>2</sub> SO <sub>4</sub> (conc.) | cubic centimeters | 1.0   |
|    | 2-hydroxy-3-aminophenazine             | grams             | 0.004 |
|    | 2:3-dimethylquinoxaline                | do                | 0.02  |
|    | Tartrazine                             | do                | 0.1   |
|    | H <sub>2</sub> O, to                   | cubic centimeters | 100   |

## Example 3

|    |                                        |                   |       |
|----|----------------------------------------|-------------------|-------|
| 50 | Potassium thiocyanate                  | grams             | 14.0  |
|    | H <sub>2</sub> SO <sub>4</sub> (conc.) | cubic centimeters | 1.0   |
|    | 2-hydroxy-3-aminophenazine             | grams             | 0.004 |
|    | 2:3-dimethylquinoxaline                | do                | 0.02  |
|    | Du-Pont Orange G, Schultz No. 39       | do                | 0.05  |
| 55 | H <sub>2</sub> O, to                   | cubic centimeters | 100   |

*Example 4*

|                            |                   |       |
|----------------------------|-------------------|-------|
| Potassium thiocyanate      | grams             | 15.0  |
| Hydrochloric acid (conc.)  |                   |       |
| cubic centimeters          |                   | 5.0   |
| 2-hydroxy-3-aminophenazine | grams             | 0.004 |
| 2:3-dimethylquinoxaline    | do                | 0.03  |
| Ferric chloride            | do                | 0.05  |
| H <sub>2</sub> O, to       | cubic centimeters | 100   |

*Example 5*

|                             |                   |       |
|-----------------------------|-------------------|-------|
| Potassium thiocyanate       | grams             | 10.0  |
| Phosphoric acid (conc.)     |                   |       |
| cubic centimeters           |                   | 1.0   |
| 2-hydroxy-3-aminophenazine  | grams             | 0.004 |
| Ferric ammonium sulphate    | do                | 0.1   |
| 2:3-dimethylquinoxaline     | do                | 0.02  |
| Potassium aluminum sulphate | do                | 3.0   |
| H <sub>2</sub> O, to        | cubic centimeters | 100   |

*Example 6*

|                           |                   |      |
|---------------------------|-------------------|------|
| Potassium thiocyanate     | grams             | 12.0 |
| Hydrochloric acid (conc.) |                   |      |
| cubic centimeters         |                   | 4.0  |
| 2:3-dimethylquinoxaline   | grams             | 4.04 |
| Ferric ammonium sulphate  | do                | 0.1  |
| H <sub>2</sub> O, to      | cubic centimeters | 100  |

*Example 7*

|                           |                   |      |
|---------------------------|-------------------|------|
| Potassium thiocyanate     | grams             | 10.0 |
| Hydrochloric acid (conc.) | do                | 4.0  |
| 2:3-dimethylquinoxaline   | do                | 0.03 |
| Potassium ferricyanide    | do                | 0.1  |
| H <sub>2</sub> O, to      | cubic centimeters | 100  |

*Example 8*

|                           |                   |      |
|---------------------------|-------------------|------|
| Potassium thiocyanate     | grams             | 10.0 |
| Hydrochloric acid (conc.) | do                | 4.0  |
| 2:3-dimethylquinoxaline   | do                | 0.03 |
| o-Nitroaniline            | do                | 0.1  |
| H <sub>2</sub> O, to      | cubic centimeters | 100  |

*Example 9*

|                                                                   |                   |      |
|-------------------------------------------------------------------|-------------------|------|
| Potassium thiocyanate                                             | grams             | 10.0 |
| Hydrochloric acid (conc.)                                         | do                | 4.0  |
| 2:3-dimethylquinoxaline                                           | do                | 0.03 |
| Ammonium vanadate (or an equivalent quantity of vanadyl chloride) | do                | 0.02 |
| H <sub>2</sub> O, to                                              | cubic centimeters | 100  |

*Example 10*

|                                              |                   |      |
|----------------------------------------------|-------------------|------|
| Potassium thiocyanate                        | grams             | 12.0 |
| Hydrochloric acid (conc.)                    |                   |      |
| cubic centimeters                            |                   | 5.0  |
| 2:3-dimethylquinoxaline                      | grams             | 0.02 |
| 1-chloro-2:4-dinitrobenzene-6-sulphonic acid | do                | 0.1  |
| H <sub>2</sub> O, to                         | cubic centimeters | 100  |

*Example 11*

|                                     |                   |      |
|-------------------------------------|-------------------|------|
| KCNS                                | grams             | 12.0 |
| Hydrochloric acid (conc.)           |                   |      |
| cubic centimeters                   |                   | 4.0  |
| 2:3-dimethylquinoxaline             | grams             | 0.03 |
| o- or m-nitrobenzene sulphonic acid | do                | 0.1  |
| H <sub>2</sub> O, to                | cubic centimeters | 100  |

*Example 12*

|                                       |                   |      |
|---------------------------------------|-------------------|------|
| Potassium thiocyanate                 | grams             | 10.0 |
| Hydrochloric acid                     | cubic centimeters | 5.0  |
| 2:3-dimethylquinoxaline               | grams             | 0.03 |
| 1-nitroanthraquinone-8-sulphonic acid | do                | 0.05 |
| H <sub>2</sub> O, to                  | cubic centimeters | 100  |

*Example 13*

|                           |                   |      |
|---------------------------|-------------------|------|
| Thiocarbamide             | grams             | 7.0  |
| Hydrochloric acid (conc.) | do                | 4.0  |
| 2:3-dimethylquinoxaline   | do                | 0.03 |
| Ferric ammonium sulphate  | do                | 0.1  |
| H <sub>2</sub> O, to      | cubic centimeters | 100  |

*Example 14*

|                         |                   |       |
|-------------------------|-------------------|-------|
| Thiocarbamide           | grams             | 5.0   |
| Sulphuric acid (conc.)  | cubic centimeters | 1.0   |
| 2:3-dimethylquinoxaline | grams             | 0.04  |
| Ammonium vanadate       | do                | 0.025 |
| H <sub>2</sub> O, to    | cubic centimeters | 100   |

*Example 15*

|                           |                   |      |
|---------------------------|-------------------|------|
| Potassium thiocyanate     | grams             | 10.0 |
| Hydrochloric acid (conc.) |                   |      |
| cubic centimeters         |                   | 4.0  |
| 2:3-dimethylquinoxaline   | grams             | 0.03 |
| p-Nitrosodimethylaniline  | do                | 0.02 |
| H <sub>2</sub> O, to      | cubic centimeters | 100  |

In Examples 13 or 14, the thiourea serves the same purpose as potassium thiocyanate.

The bleaching baths of the foregoing examples may be used, for example, for the production of dye images in a three-layer film, the emulsion layers of which respectively contain the following azo dyes:

A yellow dye which was prepared from tetrazotized toluidinedisulphonic acid coupled with 2-chloro-5-hydroxytoluene.

A magenta dye which was prepared from tetrazotized 2:5:2':5'-tetramethyl-4:4'-diaminotriphenylmethane coupled with acetyl H-acid.

A cyan dye, Fontamine Fast Green 5BL, manufactured by E. I. du Pont de Nemours and Company.

In the foregoing examples, the concentrations of each component may be varied within wide limits without seriously affecting the bleaching action of the bath, but permitting the rate of bleaching and contrast of the dye images to be adjusted as desired.

The invention is not limited to the above examples which illustrate the use of numerous oxidizing agents for oxidizing the excess of metallic silver, e. g., the ferric, vanadyl, ferri-cyanide or nitrate ions or an azo dye or a nitro or nitroso compound. Our invention comprises all modifications included within the scope of the appended claims.

We claim:

1. A method of producing a colored photographic image in a gelatino-silver halide layer containing a dye capable of being decolorized by reduction, which comprises exposing and developing the layer to produce a metallic silver image therein, and then simultaneously bleaching the dye and fixing out the silver and silver halide in a bath containing an acid bleaching agent, a mild oxidizing agent for silver, and a fixing agent.

2. A method of producing a colored photographic image in a gelatino-silver halide layer containing an azo dye capable of being decolorized by reduction, which comprises exposing and developing the layer to produce a metallic silver image therein, and then simultaneously bleaching the dye and fixing out the silver and silver halide in a bath containing an acid bleaching agent, ferric ions as an oxidizing agent for silver, and a fixing agent.

3. A method of producing a colored photo-

graphic image in a gelatino-silver halide layer containing an azo dye capable of being decolorized by reduction, which comprises exposing and developing the layer to produce a metallic silver image therein, and then simultaneously bleaching the dye and fixing out the silver and silver halide in a bath containing an acid bleaching agent, an azo dye as an oxidizing agent for silver, and a fixing agent.

4. A method of producing a colored photographic image in a gelatino-silver halide layer containing an azo dye capable of being decolorized by reduction, which comprises exposing and developing the layer to produce a metallic silver image therein, and then simultaneously bleaching the dye and fixing out the silver and silver halide in a bath containing hydrochloric acid as a bleaching agent, a mild oxidizing agent for silver, and a fixing agent.

5. A method of producing a colored photographic image in a gelatino-silver halide layer containing an azo dye capable of being decolorized by reduction, which comprises exposing and developing the layer to produce a metallic silver image therein, and then simultaneously bleaching the dye and fixing out the silver and silver halide in a bath containing an acid bleaching agent, ferric ions as an oxidizing agent for silver, and potassium thiocyanate as a fixing agent.

6. A method of producing a colored photographic image in a gelatino-silver halide layer containing an azo dye capable of being decolorized by reduction, which comprises exposing and developing the layer to produce a metallic silver image therein, and then simultaneously bleaching the dye and fixing out the silver and silver halide in a bath containing an acid bleaching agent, an azo dye as an oxidizing agent for silver, and potassium thiocyanate as a fixing agent.

7. A method of producing a colored photographic image in a gelatino-silver halide layer containing an azo dye capable of being decolorized by reduction, which comprises exposing and developing the layer to produce a metallic silver image therein, and then simultaneously bleaching the dye and fixing out the silver and silver halide in a bath containing hydrochloric acid as a bleaching agent, a mild oxidizing agent for silver, and potassium thiocyanate as a fixing agent.

8. A bleach and fixing bath for use in a bleach-out process of color photography, containing a fixing agent, a strong acid, and an azo dye as a mild oxidizing agent capable of oxidizing metallic silver to silver ion.

RICHARD V. YOUNG.  
MERRILL W. SEYMOUR.

CERTIFICATE OF CORRECTION.

Patent No. 2,322,084.

June 15, 1943.

RICHARD V. YOUNG, E<sup>m</sup> AJ..

It is hereby certified that error appears in the printed specification of the above numbered patent requiring correction as follows: Page 2, first column, line 24, for "4.04" read --0.04--; and that the said Letters Patent should be read with this correction therein that the same may conform to the record of the case in the Patent Office.

Signed and sealed this 31st day of August, A. D. 1943.

(Seal)

Henry Van Arsdale,  
Acting Commissioner of Patents.